

# UNITED STATES PATENT OFFICE.

FREDERICK E. WOODWARD, OF LACHINE, QUEBEC, CANADA.

## SHOE-FILLER.

1,136,458.

Specification of Letters Patent. Patented Apr. 20, 1915.

No Drawing.

Application filed August 8, 1913. Serial No. 783,795.

To all whom it may concern:

Be it known that I, FREDERICK E. Woodward, a citizen of the United States of America, and residing at No. 577 St. Joseph 5 street, Lachine, Province of Quebec, Dominion of Canada, have invented certain new and useful Improvements in Shoe-Fillers, of which the following is a specification.

10 The invention to be hereinafter described relates to shoe fillers.

The main objects of the invention are to provide a marketable, transportable filler which will be economical in its production 15 and use and will have the following qualities; permanent pliability, durability, waterproofness, elasticity, resiliency, softness and workability, strongly adherent to leather whether wet or dry, tenacious, low melting, 20 quick cooling, rapid setting and stable or non shifting.

At present there are two classes of fillers on the market—rubber cement fillers, and ground cork fillers. Neither of these adequately meets the demands. The first is 25 dangerous from fire and is wasteful and expensive because of evaporation, while the second requires a long time to set, involving long and expensive delays in the other 30 steps of manufacture. To fully and adequately meet all of the requirements hereinbefore enumerated the present filler has been invented.

It comprises the ingredients hereinafter 35 stated, and mixed substantially in the manner and proportions set forth in the following description. Preferably, what will be hereinafter termed the compound, is first made. This compound, which also per- 40 forms the function of a binder, is then mixed with a base of ground or granulated cork, sawdust, leather dust, or any suitable substance of like nature.

The preparation of the above filler is as 45 follows:—240 lbs. of resin is heated to the melting point in a steam jacket kettle or other suitable vessel. While it is in a hot fluid state 240 lbs. petroleum wax or wax tailings is put in, melted, and mixed. To this hot fluid 50 mixture is added 10 lbs. of bi-carbonate of soda which is stirred in until thoroughly dissolved. Into this hot fluid mass is mixed 80 lbs. of a petroleum distillate or base in the form of an oil commonly known on the 55 market as red engine oil. The oil acts on

the resin to destroy all tendency to brittleness when the mass cools and the wax greatly increases the flexibility of the resulting mixture or compound. This final compound is soft, semi-plastic, flexible, resilient, 60 elastic, non-brittle, pliable, waterproof, stable, tough, tenacious, adhesive, readily workable, low melting, quick cooling, and rapid setting. Into the hot compound above described is stirred the base material in the 65 proportion of 25 lbs. of base to 6 gals. of compound. This completes the filler. When allowed to cool it is ready for use. If desired, it may be put up in loaf form by covering the outside of each loaf with a 70 layer of the base material in well known manner, or it may be put up in barrels or boxes. A filler thus prepared is practically non-inflammable.

The heated compound and consequently, 75 the filler containing it, gives off a non-inflammable gas, thus substantially preventing combustion of the filler. Thus, in addition to the qualities previously enumerated, this filler has the additional qualities 80 of non-inflammability and smoothness and evenness in working when being molded into the cavity.

The ingredients above named are common 85 trade articles and, therefore, vary more or less in purity. Consequently their proportions will vary somewhat on that account. Likewise, the requirements of the filler for use in summer are different than the requirements for winter. For that reason, the 90 proportions will be varied. Thus, for winter use, for instance, there would be a greater quantity of oil than for summer use. Obviously, other ingredients having either individually or collectively, similar properties may be used for those specifically mentioned. Many of these are well known on 95 the market and would readily occur to any one skilled in the art to which this invention relates. Therefore, they need not be set forth here.

Having fully set forth and described my invention, what I claim and desire to protect by Letters Patent of the United States.

1. A permanently tenacious, quicksetting, 105 permanently elastic, non-inflammable shoe filler capable of being molded into a thin pliable layer filling the shoe bottom, said filler comprising, wax tailings, resin, petroleum oil, a comminuted resilient solid ma- 110

- terial and a substance which when combined with said ingredients and heated, gives off a non-inflammable gas.
2. A shoe filler consisting of wax tailings, resin, petroleum oil, a substance which when incorporated in the completed filler will give off non-inflammable gas upon heating of the filler, and a comminuted resilient solid material.
- 10 3. A shoe filler consisting of wax tailings, resin, petroleum oil, bi-carbonate of soda, and a comminuted resilient solid material.

4. A shoe filler consisting of wax tailings 240 lbs. resin 240 lbs. petroleum oil 15 80 lbs. bi-carbonate of soda 10 lbs. and a comminuted resilient solid material in the proportion of 25 lbs. of comminuted resilient solid material to 6 gals. of the above mixture.

Signed this 31st day of July, 1913, in the presence of two witnesses.

FREDERICK E. WOODWARD.

Witnesses:

GEORGE H. CROSS,  
RICHARD E. WOODWARD.